

Feb. 26, 1952

R. B. HARLAN ET AL

2,587,152

METHOD OF DECORATING CERAMIC BODIES

Filed Jan. 7, 1949

*Fig. 1*



*Fig. 2*



*Fig. 3*



*Fig. 4*



INVENTORS,  
RICHARD B. HARLAN and  
WALTER E. GARDNER

BY *John Brown*,

ATTORNEY.

## UNITED STATES PATENT OFFICE

2,587,152

## METHOD OF DECORATING CERAMIC BODIES

Richard B. Harlan, Long Beach, and Walter E. Gardner, Whittier, Calif., assignors, by mesne assignments, to Ceratile Corporation, Paramount, Calif., a corporation of California

Application January 7, 1949, Serial No. 69,644

6 Claims. (Cl. 117—40)

1

The present invention relates to a method and means whereby ceramic bodies of any character, specifically by way of example, tile, may be surface decorated, the decoration being in the glaze.

With our method, various decorative effects may be obtained which add to the beauty of the tile in that the surface of the tile may be in color or a plurality of colors, or certain designs may be in one color, while other designs are in a different color, with all of the colors of a controlled nature in that colors may be brilliant or pastel, as desired.

An object of the invention is to reduce the number of steps necessary to decorate a ceramic body and wherein superior results are obtained after firing the body.

A further object is the provision of a method of decorating ceramic bodies wherein embossed effects are attained in the design or background.

We have discovered that a glazed design may be applied to a ceramic body followed by applying a further glaze or a background glaze thereover, which glazes after glost firing will not materially fuse or run together, but tend to separate so as to produce unusual effects, although predetermined, in the glaze decoration.

We are aware that prior to our invention, various methods have been utilized in the art to decorate ceramic bodies, among which may be mentioned the adding of coloring oxides to the glaze; the so-called underglaze method which utilizes slip painting or underglaze colors, and sometimes underglaze decalcomania; the overglaze method which utilizes overglaze colors and overglaze decalcomania, and the inlay method which utilizes full glazes applied by hand.

Those skilled in the art to which this invention belongs, will recognize these different methods now in use for the decoration of ceramic articles and the difficulties attendant in such decoration. Briefly some of these difficulties are as follows: in overglaze work three firings are necessary and overglaze work is not durable or wear-resistant; in underglaze work deep rich colors are not easily obtained and of a necessity the glaze used must be transparent, and the inlay method is done by hand which is expensive, and results in ununiformity on work.

A further object of our invention is a decoration method for ceramic articles which is inexpensive in actual practice, does not of necessity require skilled labor, wherein uniform results are attained, and which is simple to practice. Furthermore, the glaze decoration is durable and wear-resistant, and all the beauty of the design is preserved.

2

In the drawing,

Figure 1 is a section of a plain tile;

Figure 2 is a sectional view of the tile of Figure 1, with a glazed design applied thereto;

Figure 3 is the tile of Figure 2 with a background glaze applied over the design glaze and the surface of the tile; and

Figure 4 is a sectional view showing the appearance of the design glaze, and the background glaze after glost firing.

Primarily for the purpose of the present invention, we have assumed a classification for glazes. Searle in The Encyclopaedia of the Ceramic Industry states as to glaze compositions; (1) glazes are often divided broadly into lead glazes and leadless glazes, and they may be classified according to their composition, i. e. as to the nature of the flux; (2) the alumina to silica ratio or the acid to base ratio; and (3) the acidity number or acid equivalent. We accept this classification for an understanding of the present invention and it is adopted for the reason that the same classification is used for glass. We, therefore, for the purpose of illustrating our invention, classify the glazes into four types:

The above listed types of glazes are well known to those skilled in the art and constitute recognized glaze types. By referring to "An Encyclopaedia of the Ceramic Industries" by Searle, published 1930, we find in Volume II on pages 251 and 252 and also on page 248 under the title "Lead glaze" a discussion of the lead silicate glazes, and as this publication indicates the lead silicate glazes comprise essentially a mixture of lead oxide and silica. The proportions of the materials may vary throughout extremely wide ranges, there being substantially no limit. Some compositions having as low as 1% silica are described, and the article indicates that the quantity of silica varies the melting point. The publication clearly shows that the ratio of lead oxide to silica merely affects the refractoriness and softening temperatures of the glaze. On page 248 the publication states: "The use of a suitable proportion of lead in a glaze has the following results: (a) It makes the molten glaze mobile, so that it flows easily over the surface of the ware and produces a more uniform coverage than a less mobile glaze; (b) It produces a glaze of high refractivity and therefore imparts greater lustre; (c) It produces glazes having so great a range of fusibility that small variations in the composition of the glaze are of much less importance and are far less likely to cause trouble than when no lead is present." This article further states; "The addition of silica, alumina,

lime, potash, etc. raises the melting point of the glaze and makes a harder product." Also in Volume II on page 250 the author describes the effect of changes in proportion of lead oxide on the maturing time and points out that an excess of silica or alumina will raise the melting point.

The second type of glaze described above namely, lead-boro-silicates, are discussed on page 113 of Volume I of the Searle Encyclopaedia. Under the definition of Boracic glazes, Searle states that the glazes containing boric oxide may or may not contain lead oxide also. Those glazes containing both boric oxide and lead oxide are commonly referred to as lead-boro-silicates (see technological papers of the Bureau of Standards, No. 31, published 1914, page 4).

The alkali-boro-silicate type of glaze is discussed in Searle, Volume II, page 252 under "leadless glazes" and defines those glazes containing no lead oxide but containing alkali oxides instead. The article states that these glazes may have their fusibility regulated by the addition of borax, boric acid, soda or potash. The alkali glazes containing boric acid are the alkali-boro-silicate glazes contemplated by applicant.

Page 113 of Volume II of the Searle Encyclopaedia defines alkaline-calcerous glazes, which is the glaze identified herein as the alkali-lime-silicate glaze type 4 above. Under (D) Searle identifies a group of such calcareous glazes in which the flux is lime.

Throughout the entire published literature and particularly that identified above the art recognizes the classifications heretofore set forth and clearly shows that it is within the skill of the art to compound glazes within those classifications. It is well within the knowledge of the art that the materials constituting each type must be present in significant quantities and, as the literature indicates, the relative proportions vary certain characteristics of the glaze, all as is well known. Throughout this application and claims it is to be understood that identification of any one of the types refers to glazes comprising essentially substantial proportions of the named ingredients in the oxide form.

1. Lead-silicate glazes.
2. Lead-boro-silicate glazes.
3. Alkali-boro-silicate glazes.
4. Alkali-lime-silicate glazes.

We make use of this glaze classification, in the practice of our invention and wherein we utilize a glaze of one classification as the design glaze, and a glaze of another classification for the background glaze. In other words, we may utilize one or more glazes in the same classification as design glazes, and a different type of glaze for the background. This holds true at all times in the practice of our invention. Hence, we may utilize one or more types of glazes for the design provided a different type of glaze is used for the background. If glazes of the same type are in contact, the glazes may run together.

The glazes may be prepared in any usual manner, such as by ball milling the materials used in the glaze composition with water. One method which we have employed is to dry out the design glaze or glazes to be used, and then suspend the glaze in an oil medium followed by passing the glaze through a color mill to insure homogeneity.

Referring to the drawing, assuming a design glaze of one of the glaze types previously mentioned, the design may be applied to the surface

of the ceramic article, specifically the tile by passing the design glaze through a coarse silk screen carrying the desired design. The design glaze may also be applied by brushing or spraying or by any other common method of applying a glaze to a ceramic article in the form of a design. After the design glaze has dried at room temperature, the background glaze may be dipped or sprayed over the surface of the tile and the design glaze, as shown in Figure 3. Thereafter, the tile is glost fired. Drying of the design glaze before application of the background glaze is desirable for handling reasons, although such procedure is not necessary if care is exercised.

The background and design glazes mature in the same temperature range or in an overlapping temperature range. Therefore, the method of our invention is limited in temperature only to the extent that specified types of glazes can be used together. By way of example and not in limitation of the invention, an upward firing limit of glazes containing either lead or boron, or both, is approximately Seger cone 5, or about 1190° C. (2174° F.). The lower limit of an alkali-lime-silicate glaze is Seger cone 1, or about 1100° C. (2012° F.), and an alkali-boro-silicate glaze, cone 014 or 815° C. (about 1500° F.). The lower limit for the lead and boron glazes is approximately Seger cone 08 or about 945° C. (1733° F.). The upper limit for the alkali-lime-silicate glaze is about Seger cone 3 or about 1145° C. (2093° F.), and the upper limit for an alkali-boro-silicate glaze is about Seger cone 02, or about 1095° C. (2003° F.).

We have found that if the design glaze is more fluid or has less viscosity than the background glaze, the background glaze will readily flow or separate from the design glaze during the glost firing, due to the lessening of the surface tension between the two glazes. Hence, the viscosity of each glaze is utilized as a means of controlling the degree of separation therebetween. This separation is illustrated in Figure 4 and wherein the design glaze is shown at 1, and the background glaze at 2, the background glaze having separated from the design glaze, as shown at 3. This separation is quite marked in actual practice. The viscosity of the glaze may be controlled by the alumina content thereof or by increasing the refractoriness of the glaze by the addition of refractory oxides, such as magnesium oxide, calcium oxide, and others. This latter method affects the maturing temperature of the glaze, but so long as the maturing temperature of one glaze is within the maturing range of the other glaze, satisfactory results are obtained. Obviously, the viscosity may be lessened by the addition of more fluxing oxides in the glaze composition.

The Searle Encyclopaedia previously identified, in Volume II on pages 114 and 115 describes at some length the effects of alumina in glazes and indicates that the addition of alumina to a glaze composition has the effect of increasing its viscosity.

We have found that the thickness of the application of the glazes is of importance, and that the design glaze should not be appreciably thicker than the background glaze. In practice, the range of thickness for the design glaze may be from 3 to 20 thousandths, while the background glaze may vary from 5 to 25 thousandths. To obtain embossed design effects, the design glaze may be one-half as thick as the background glaze.

As an illustration of formulas for design and background glazes which may be utilized, we give the following examples:

#1. Design glaze—(lead-boro-silicate type)

Maturing range—cone 07 to 05

|           |                                     |                                     |
|-----------|-------------------------------------|-------------------------------------|
| .175 NaKO |                                     | .522 B <sub>2</sub> O <sub>3</sub>  |
| .162 CaO  |                                     | .123 Fe <sub>2</sub> O <sub>3</sub> |
| .575 PbO  | .298 Al <sub>2</sub> O <sub>3</sub> | .350 SnO <sub>2</sub>               |
| .087 CuO  |                                     | 1.905 SiO <sub>2</sub>              |

.999

#1-B. Background glaze (alkali-boro-silicate)

Maturing range—cone 06 to 04

|            |                                     |                                    |
|------------|-------------------------------------|------------------------------------|
| .7330 NaKO |                                     | .378 B <sub>2</sub> O <sub>3</sub> |
| .1775 ZnO  | .375 Al <sub>2</sub> O <sub>3</sub> | .109 ZrO <sub>2</sub>              |
|            | 0.22 Sb <sub>2</sub> O <sub>3</sub> | .080 NaF                           |

.8905

2.64 SiO<sub>2</sub>

#2. Design glaze—(lead-silicate type)

Maturing range—cone 08 to 05

|                        |                                     |                       |
|------------------------|-------------------------------------|-----------------------|
| .716 PbO               |                                     |                       |
| .011 K <sub>2</sub> O  |                                     |                       |
| .030 Na <sub>2</sub> O | .049 Al <sub>2</sub> O <sub>3</sub> | .921 SiO <sub>2</sub> |
| .206 CuO               |                                     |                       |

.963

#2-B. Background glaze (lead-boro-silicate type)

Maturing range cone 06 to 04

|                        |                                     |                                    |
|------------------------|-------------------------------------|------------------------------------|
| .118 Na <sub>2</sub> O |                                     |                                    |
| .006 K <sub>2</sub> O  |                                     |                                    |
| .490 PbO               | .328 Al <sub>2</sub> O <sub>3</sub> | .215 SiO <sub>2</sub>              |
| .291 ZnO               |                                     | .523 B <sub>2</sub> O <sub>3</sub> |
| .094 CuO               |                                     | .337 ZrO <sub>2</sub>              |

.999

#3. Design glaze (lead-boro-silicate type)

Maturing range—cone 1 to 5

|                        |                                     |                                    |
|------------------------|-------------------------------------|------------------------------------|
| .125 Na <sub>2</sub> O |                                     |                                    |
| .272 CaO               |                                     |                                    |
| .047 K <sub>2</sub> O  |                                     | .250 B <sub>2</sub> O <sub>3</sub> |
| .300 ZnO               | .198 Al <sub>2</sub> O <sub>3</sub> | 2.060 SiO <sub>2</sub>             |
| .070 CuO               |                                     | .167 ZrO <sub>2</sub>              |
| .248 PbO               |                                     |                                    |

.962

#3-B. Background glaze (alkali-lime-silicate)

Maturing range (cone 1 to 5).

|                        |                                     |                                    |
|------------------------|-------------------------------------|------------------------------------|
| .135 Na <sub>2</sub> O |                                     |                                    |
| .693 CaO               |                                     | .266 B <sub>2</sub> O <sub>3</sub> |
| .232 K <sub>2</sub> O  | .380 Al <sub>2</sub> O <sub>3</sub> | 3.340 SiO <sub>2</sub>             |
| .049 ZnO               |                                     | .354 ZrO <sub>2</sub>              |

By referring to "Ceramic Glazes" by Cullen W. Parmelee, published in 1948, there will be found beginning on page 6 thereof a discussion of opacifiers and identification of the various materials commonly employed for such purpose. The chapter beginning on page 268 of Parmelee discusses coloring materials and identifies the various materials commonly used for imparting various colors to glazes.

The Parmelee publication, beginning on page 125, also discusses the effects of the addition of various materials on the maturing of glazes and again on page 27 shows the effect of alumina on the refractoriness and maturity of a glaze. This publication shows that it is well known to those skilled in the art that color and opacity of a glaze may be controlled and that the maturing range may also be adjusted by well known and described procedures. Thus it will be apparent to those skilled in the art that each of the examples described above contains as its essential constituents, the oxides indicated by the titles

thereof. It will also be apparent to those skilled in the art that the examples contain opacifiers and coloring oxides.

Attention is called to the fact that where we have designated one glaze as "design" and the other glaze as "background," that these designations may be reversed as long as the principle of the invention, as outlined heretofore is followed.

10 The ceramic bodies may be decorated rapidly and uniformly by one operator applying the design glaze, followed by a second operator applying thereover, after the design glaze has dried, the background glaze by spraying or any other method. This results in the so-called straight line application of glazes and is rapid and economical from a labor standpoint. Given glazes of definite classes with a given firing temperature, the results are always the same and the tile so treated will be substantially uniform in design and color. It is a feature of the invention that the separation of the glazes occurs without any noticeable irregularity during the glost firing. Each piece of tile or other ceramic article will have an almost identical fired appearance with another tile of the same type providing it is treated in the same or a like manner.

We claim:

1. In a method of producing decorated ceramic clay articles, the steps of; applying a first alumina-containing glaze-forming composition to selected portions of a surface of said article, said composition having sufficient solids to form a substantially uniform layer of solids of a thickness of from 3 to 20 thousandths of an inch before firing, thereafter applying a continuous layer of a background glaze-forming composition containing alumina over said first layer and uncoated portions of said surface, said background layer having sufficient solids to form a substantially uniform layer of solids of a thickness of from 5 to 25 thousandths of an inch before firing, and simultaneously glost firing said first and background compositions on said article; each of said first and background compositions being selected from the group consisting of: (1) a lead-silicate glaze consisting essentially of substantial proportions of lead oxide and silica, (2) a lead-boro-silicate glaze consisting essentially of substantial proportions of lead oxide, boron oxide and silica, (3) an alkali-boro-silicate glaze consisting essentially of substantial proportions of alkali metal oxides, boron oxide and silica and (4) an alkali-lime-silicate glaze consisting essentially of substantial proportions of alkali metal oxides, calcium oxide, and silica; said first and background compositions each being a different one of said group and said first composition having substantially less alumina than said background composition whereby during glost firing said background composition develops a fluid state of lesser fluidity than that of said first composition and withdraws therefrom without substantial diffusion thereinto to uncover said first composition on said selected portions, both said compositions having overlapping maturing temperature ranges and said glost firing being carried out within said overlapping ranges.

2. A method as defined in claim 1 wherein said first composition contains ceramic pigmenting materials.

3. A method as defined in claim 1 wherein said first composition contains ceramic pigmenting materials and wherein said background composition contains opacifying materials.

4. A method as defined in claim 1 wherein said first composition is a lead-boro-silicate glaze and wherein said background composition is an alkali-boro-silicate glaze.

5. A method as defined in claim 1 wherein said first composition is a lead-silicate glaze and wherein said background composition is a lead-boro-silicate glaze.

6. A method as defined in claim 1 wherein said first composition is a lead-boro-silicate glaze and wherein said background composition is an alkali-lime-silicate glaze.

RICHARD B. HARLAN.  
WALTER E. GARDNER.

#### REFERENCES CITED

The following references are of record in the file of this patent:

#### UNITED STATES PATENTS

| Number    | Name     | Date          |
|-----------|----------|---------------|
| 488,683   | Vollrath | Dec. 27, 1892 |
| 529,670   | Stewart  | Nov. 20, 1894 |
| 2,019,676 | Hommel   | Nov. 5, 1935  |